

Patented Jan. 12, 1926.

1,569,578

# UNITED STATES PATENT OFFICE.

OTTO RÖHM, OF DARMSTADT, GERMANY.

MANUFACTURE OF TANNING SUBSTANCES.

No Drawing.

Application filed March 5, 1924. Serial No. 697,155.

To all whom it may concern:

Be it known that I, OTTO RÖHM, doctor of philosophy, director, a citizen of the German Republic, residing at Darmstadt, 5 Germany, have invented certain new and useful Improvements in the Manufacture of Tanning Substances, of which the following is a specification.

My invention relates to an improved tanning method and more particularly to a new and useful tanning liquor or substance and the process of manufacturing the same, the essential constituents of the latter being an iron salt, an alkali metal silicate and sulfite cellulose liquor.

In manufacturing the tanning substance or liquor according to my invention I employ the three ingredients either in a liquid form or in a dry state. In the former case 10 I mix in the proportions required a solution of an iron salt with a solution of an alkali metal silicate and a more or less diluted sulfite cellulose liquor in order to obtain a tanning liquor of suitable composition, and in the latter case I mix the dry or dried substances together and dissolve the mixture in a suitable solvent. In some cases it may be advisable to employ, for example, two of the three substances in a 15 dry state and to dissolve them, after they have been intimately mixed together, in the third substance which is in the form of a solution of appropriate concentration.

In employing a thus prepared liquor for 20 tanning purposes, the hides or skins may be treated therewith in any suitable manner and in accordance with any appropriate operations hitherto known in the art. In particular I have found that especially thick 25 hides and skins can be profitably treated with my improved tanning liquor and heavy leather of best quality can be produced thereby. A particular advantage further resides in the fact that the tanning 30 operation ensures good weight which is mainly due to a high proportion of iron 35 oxid and silicic acid retained in the leather. The latter is of a grainy structure and of a 40 light brown colour similar to that of oak-bark tanned sole-leather. The colour is 45 lighter and more uniform than in cases 50 where iron salt and sulfite cellulose liquor alone are used for tanning purposes. Evidently the presence of silicic acid has a 55 clearing and filling effect.

It has been suggested heretofore to pro-

duce so-called iron leather by tanning the 60 hides or skins with the aid of iron oxid or iron salts containing a strong acid, and sulfite cellulose liquor, and to carry out the 65 tanning process either in a single operation by treating the skins and hides with a mixture of the iron compound and the liquor, or in two operations by treating the same 70 first with the iron compound and subsequently with the liquor. Further it has been recommended heretofore to employ for 75 tanning purposes sulfite cellulose liquor mixed with substances other than iron compounds. Furthermore it has been suggested 80 some time ago to use iron silicate for tanning purposes.

In contradistinction to the prior art, my 85 invention contemplates the new idea of employing a tanning liquor containing three 90 well defined ingredients, that is to say, an iron compound or compounds, a silicate or silicates and sulfite cellulose liquor or, in other words, an iron salt solution, a silicate solution and sulfite cellulose liquor 95 and, accordingly, my improved tanning method is in principle novel inasmuch as therein, for the first time, the aforesaid three ingredients or constituents are united 100 in a suitable manner and with the result of ensuring thereby certain new and important advantages over the old state of the art.

Apart from the aforesaid advantages 105 of my method of producing leather of superior qualities, it has been found that the 110 defects of the methods of tanning hides and skins with the aid of iron solutions, as hitherto suggested or practiced, are entirely remedied by my new method. A further advantage thereof, moreover, resides in the 115 fact that the tanning liquor prepared in accordance with my invention is of practically imperishable nature and further, that the percentage of iron silicate therein may be increased to a relatively high degree 120 without the occurrence of precipitation.

In carrying out my method of making a 125 tanning liquor and of treating hides and skins with such liquor I proceed in a preferable way as follows:

I add to 50 kg. of sulfite cellulose liquor of 20° Bé., 20 kg., of a 50% solution of iron chloride and a solution of 25 kg. water-glass of 36° Bé. in 125 litres of water. The 130 solution thus obtained is sufficient for tanning 100 kg. of cowhides which are soaked

therein and dressed for about three days in a suitable dressing trough.

The tanning operation, properly speaking, thus accomplished, the hides are washed in water, subsequently treated with an appropriate oil and finished in the customary manner to sole-leather.

What I claim is:—

1. The method of manufacturing a tanning substance, consisting in mixing together an iron salt, an alkali metal silicate and sulfite cellulose liquor, substantially as described.
2. The method of manufacturing a tanning liquor, consisting in mixing together a solution of an iron compound or compounds, a solution of an alkali metal silicate or silicates and sulfite cellulose liquor, substantially as described.
3. The method of manufacturing a tanning liquor consisting in mixing together an iron compound or compounds, an alkali metal silicate or silicates and dry sulfite cel-

lulose liquor, and dissolving the mixture in a suitable solvent, substantially as described.

4. A tanning substance consisting of an iron compound or compounds, an alkali metal silicate or silicates and dried sulfite cellulose liquor mixed together in the proportions required for the purpose.

5. A tanning liquor consisting of an iron compound or compounds, an alkali metal silicate or silicates and sulfite cellulose liquor mixed and dissolved in water in the proportions required for the purpose.

6. The method of manufacturing a tanning substance, consisting in mixing together a solution of iron chloride, a solution of water-glass and sulfite cellulose liquor.

7. A tanning substance, consisting of iron chloride, water-glass and sulfite cellulose liquor.

In testimony whereof I affix my signature.

OTTO RÖHM.